

## UNITED STATES PATENT OFFICE

2,613,192

## POLISHING COMPOSITION

Herbert Honig, New York, N. Y.

No. Drawing: Application October 21, 1947;  
Serial No. 781,251

2 Claims. (Cl. 260—29.3)

1

This invention relates to a polishing and finishing compound for restoring and revitalizing the finishing coat of furniture, woodwork and surfaces of articles made from metal, plastic and similar material.

It is an object of the invention to provide a compound for application to varnished, shellac-coated, glazed, painted or other surfaces of articles for polishing and finishing the same, which compound may be used for impregnating and saturating cloth which forms the carrier for said compound.

A further object of this invention is to provide as an applicator a loosely woven and soft-textured flannel or similar cloth material which is chemically treated with the polishing or finishing composition to such an extent that it always remains damp and is ready for polishing operation with the required amount of composition and contains preferred ingredients which will be substantially kept in the cloth during and after use.

A further object of the invention is to provide a cloth of the aforesaid nature which may be kept in a closeable container to prevent the cloth from drying out when not in use.

Still another object of this invention is to provide means facilitating the treatment of wooden, metallic and other surfaces, either lacquered, varnished, shellac-coated, enameled or painted which, upon application of the impregnated cloth will be cleaned, polished and disinfected.

Still another object of this invention is to provide means for producing a glossy and long lasting polish on the aforesaid surfaces which, when worked upon by means of the new compound will also be subjected to cleaning, filling in and hardening actions.

In accordance with the present invention, the character of the original finishing substances used for wood is substantially approached in the present compound or substance incorporated in the cloth or similar carrier so that the polishing operation becomes substantially equivalent to the finish applied to the article after its manufacture.

Principally, the invention aims at a new composition of matter and its incorporation in a cloth or similar carrier which composition includes a plastic finishing agent which is capable of being uniformly applied to the cloth carrier, is economical in use and instantaneously ready for application to suitable surfaces, said composition being transferred onto the respective surfaces by rubbing it briskly e. g. on the surface of woodwork (if worn out places thereof are to

be restored to previous lustre), or merely by wiping the woodwork surfaces evenly and gently (if the same are to be finished, polished or revitalized).

5 The new compound further includes an agent for removing dirt spots and affords, through simple application, the cleaning and removal of undesired spots caused by dirt, a gradual filling-up of cavities caused by scratches and hardening 10 of the polished surfaces upon exposure thereof to the atmosphere. In its removing and cleaning operations, the compound possesses the remarkable faculty of making use of the dust and other foreign matter which it encounters during application and utilises the grit and other abrasive substances which may be found in the dust to scour and to remove stains, discolorations and surface-embedded dirt.

In addition to these effects, the compound 15 made in accordance with this invention imparts certain disinfecting and insect-repellent properties to the articles to which it is applied so that the compound and/or the cloth treated therewith may be safely used in cleaning of medical equipment or apparatus.

25 Other objects of the invention will appear as the description proceeds; it being understood, however, that it is not intended that the invention be limited to the exact details described herein; and it is further intended that there 30 be included as part of the invention all such obvious changes and modifications thereof as would occur to a person skilled in the art to which this invention pertains and as would fall within the scope of the claims.

35 The compound may preferably consist of the following ingredients in the following proportionate relationship:

|                                                                                                                                           | Per cent  |
|-------------------------------------------------------------------------------------------------------------------------------------------|-----------|
| 40 Synthetic resin of the phenol type, such as a phenol-formaldehyde resin containing a thinning substance in the form of a resin varnish | 10 to 15  |
| Liquid soap, such as pine oil soap with chlorophyll                                                                                       | 10 to 14  |
| 45 With the addition of turpentine                                                                                                        | 8 to 10   |
| Vegetable and mineral oils, such as lemon oil                                                                                             | 15 to 20  |
| And/or paraffin oil                                                                                                                       | 15 to 20  |
| Acetic acid                                                                                                                               | 12 to 16  |
| 50 Alcohol, such as butanol                                                                                                               | 5 to 8    |
| Ammonia softened water                                                                                                                    | remainder |

The cloth used as a carrier may be in the form of cheesecloth or soft flannel which is impregnated with the aforesaid composition and then enclosed in a container during non-use.

Of the aforesaid ingredients of the compound, the most important one is the special varnish containing phenol formaldehyde resin which is so composed that it dries upon being exposed for a relatively long period of time to the atmosphere. The quality of the composition is such that it remains in condition for use over a long period of time when preserved in a closed container.

The cloth may be used as though it were an ordinary polishing cloth but instead of merely polishing the work surface, it actually provides a finish thereon which possesses an affinity to varnish, lacquer or similarly treated work surface.

It is well understood that deodorants and scent-improving or perfume substances of known description may be added to the compound.

It can thus be seen that there has been provided according to the invention as a new composition of matter, a polishing agent, comprising in combination a thinned phenol-formaldehyde resin, a liquid soap with the addition of turpentine, said phenol-formaldehyde resin and said liquid soap being present within said agent in substantially equal amounts, lemon oil, and paraffin oil each in substantially equal amounts, but larger than the amount of each of said phenol-formaldehyde resin and of said liquid soap, the amount of said turpentine being smaller than that of said phenol-formaldehyde resin and said liquid soap, and further a cleansing vehicle containing a mixture of acetic acid and alcohol, the remainder being water.

The several ingredients hereinabove referred to which impart certain properties to the polishing cloth, such as cleaning (dirt removing), hardening and other desired effects, are illustrative of the formula forming the subject matter of this invention.

Having thus described the invention, what is claimed as new and desired to be secured by Letters Patent, is:

1. As a new composition of matter, a polish-

ing agent, comprising, in combination, resin varnish containing phenol-formaldehyde resin ranging from 10 to 15% by weight, a liquid soap in the form of chlorophyl containing pine oil soap ranging from 10 to 14% by weight, whereby said formaldehyde resin and said soap are present within said agent in substantially equal amounts, 8 to 10% by weight of turpentine, 15 to 20% by weight of lemon oil with the addition of paraffin oil amounting to 15 to 20% by weight, whereby said lemon oil and said paraffin oil are present within said agent in substantially equal amounts and each being present in a larger amount than that of each of said phenol-formaldehyde resin and of said soap, and with the further addition of a cleansing vehicle consisting of a mixture of acetic acid in the amount of 12 to 16%, and alcohol in the amount of 5 to 8%, the remainder being water.

2. As a new composition of matter, a polishing agent, comprising, in combination, resin varnish containing phenol-formaldehyde resin ranging from 10 to 15% by weight, a liquid soap in the form of chlorophyl containing pine oil soap ranging from 10 to 14% by weight, whereby said formaldehyde resin and said soap are present within said agent in substantially equal amounts, 8 to 10% by weight of turpentine, 15 to 20% by weight of lemon oil, and with the further addition of a cleansing vehicle consisting of a mixture of acetic acid in the amount of 12 to 16%, and alcohol in the amount of 5 to 8%, the remainder being water.

HERBERT HONIG.

#### REFERENCES CITED

The following references are of record in the file of this patent:

#### UNITED STATES PATENTS

| Number    | Name           | Date          |
|-----------|----------------|---------------|
| 1,809,970 | Holland et al. | June 16, 1931 |
| 2,399,693 | Ratner         | May 7, 1946   |
| 2,411,938 | Ratner         | Dec. 3, 1946  |